

March 12, 1935.

P. McL. GINDER ET AL

1,994,357

PURIFYING ZINC

Filed May 26, 1933

2 Sheets-Sheet 1



INVENTORS

Philip McLean Ginder  
Willie McClelland Ginder

BY Robert Kerr Waring

Pennie, Davis, Mann & Edmunds

ATTORNEYS

March 12, 1935.

P. McL. GINDER ET AL

1,994,357

PURIFYING ZINC

Filed May 26, 1933

2 Sheets-Sheet 2



Fig. 5,



Fig. 4,



INVENTORS

Philip McLean Ginder  
Willis Mc Donald Pearce

BY Robert Kerr Waring

Pennie, Davis, Marin - Edmonds

ATTORNEYS

## UNITED STATES PATENT OFFICE

1,994,357

## PURIFYING ZINC

Philip McLean Ginder, Willis McGerald Peirce,  
and Robert Kerr Waring, Palmerton, Pa., as-  
signors to The New Jersey Zinc Company, New  
York, N. Y., a corporation of New Jersey

Application May 26, 1933, Serial No. 672,998

2 Claims. (Cl. 75—28)

This invention relates to purifying zinc metal by distillation, and has for its object the provision of an improved method of and apparatus for producing purified zinc vapor from zinc metal 5 contaminated with both lead and cadmium, or other metallic impurities of higher and lower boiling points than zinc. Throughout this specification and the appended claims, lead and cadmium are taken as representative of metal impurities of higher and lower boiling points, respectively, than zinc, and it is therefore to be understood that specific mention of lead and cadmium in the specification and claims is illustrative and not restrictive.

15 In our copending application for Letters Patent of the United States, Ser. No. 620,634, filed July 2, 1932, we have disclosed a method of and apparatus for removing cadmium and the like from zinc metal by fractional distillation in a rectifying column. In another copending application for Letters Patent of the United States, Ser. No. 668,314, filed April 28, 1933, we have disclosed a novel and advantageous combination of our method of cadmium elimination with the method 20 of eliminating lead from zinc metal by the rectifying action of a reflux column described in the copending application of Messrs. Holstein and Ginder, Ser. No. 540,566, filed May 28, 1931. Our present invention involves a further novel and 25 advantageous combination of these methods of removing lead and cadmium from impure zinc metal by fractional distillation in a rectifying column, and is characterized by first subjecting the impure molten zinc metal to a rectification treatment for the removal of cadmium and then subjecting the so-treated impure molten zinc metal to a second rectification treatment for the 30 removal of lead, whereby purified zinc vapor is obtained. Thus, the present invention involves 35 subjecting zinc metal contaminated with lead and cadmium to two successive rectification treatments in the first of which molten zinc metal purified with respect to cadmium is obtained and delivered to the second rectification treatment from 40 which zinc vapor purified with respect to lead is obtained. The purified zinc vapor may be directly burned for the production of zinc oxide, or may be condensed as zinc dust, or utilized in any other desired manner.

45 The invention may be carried out in various forms and types of apparatus. We have illustrated in the accompanying drawings an apparatus particularly adapted for the practice of the invention. In the drawings

50 Fig. 1 is a sectional elevation of the apparatus,

Figs. 2, 3 and 4 are explanatory sectional views on the section lines 2—2, 3—3 and 4—4, respectively, of Fig. 1, and

Fig. 5 is a detailed sectional view on the section line 5—5 of Fig. 4.

Referring to Fig. 1 of the drawings, there is shown an upright furnace structure 10 having a heating chamber or laboratory 11 provided with burner openings 12 and an outlet (not shown in the drawings) near the top thereof for the exhaust heating gases. It will, of course, be understood that any other appropriate means of heating may be used in lieu of the burners and hot gases of combustion indicated in the drawings.

The lower portion of a cadmium-eliminating 15 rectifying column (hereinafter designated cadmium column) is built within the heating chamber 11. This lower portion of the column is built up of rectangular trays or pots 13 of silicon carbide or equivalent refractory material of good 20 heat conductivity. The top and bottom edges of the trays are bevelled as at 14 so that they may be stacked one above the other to form an upright or vertical column. The joints between the 25 trays are made zinc-vapor-tight by an appropriate cement, such as a cement of silicon carbide with a small amount of clay. Each tray 13 has a V-shaped peripheral trough or channel 15 for holding molten metal. This trough is formed between the outer wall of the tray and an inner inclined wall 16 of the bottom 17 of the tray. Each tray 13 is an integrally molded article. The bottom 17 has an opening 18 approximate one end thereof, and the upper edge of the opening has a rib 19 for retaining a shallow layer of molten metal on 30 the top surface of the bottom member 17 (see Fig. 3).

The trays 13 are stacked in staggered relationship with respect to the openings 18 so that the bottoms thereof form a column of superposed and 35 vertically spaced baffles through which vapor ascends and molten metal descends in tortuous or zig-zag paths.

The upper portion of the cadmium column is built up of superposed rectangular trays 20 of 40 silicon carbide or the like, with the top and bottom edges bevelled as in the case of the trays 13, and the joints between trays made zinc-vapor-tight with cement. The bottom of each tray 20 has a transverse opening 21 approximate 45 one end thereof, and its upper surface is provided with spaced transverse ribs 22 parallel to the opening 21, the ribs being of progressively increasing height from the end nearest the opening to the end furthest therefrom. The trays 20

5

10

15

20

25

30

35

40

45

50

55

are stacked in staggered relationship with respect to the openings 21 (see Fig. 3). Above the furnace structure 10, the column of trays 20 is surrounded by an appropriate layer of insulating material 23.

The bottom of the lowermost tray 20 approaches very close to the bottom of the uppermost tray 13, and the space between these trays available for vapor flow is consequently relatively narrow. For this reason the opening 21' in the lowermost tray 20 is directly above the opening 18 in the uppermost tray 13, so that vapor can ascend directly through these two openings. The inner edge of the opening 21' has an upstanding rib or lip 29 terminating short of the sides of the tray to direct molten metal overflowing the tray into the troughs of the tray beneath, as more fully explained in connection with the similar arrangement illustrated in Fig. 5.

20 The cadmium column is surmounted by a condenser or dephlegmator 24. The amount of condensation in the dephlegmator is controlled by heat insulation in appropriate amount. Molten metal condensing in the dephlegmator flows back 25 into the cadmium column by passing under a curtain wall 25 and over a dam 26. The curtain wall 25 acts as a skimmer to prevent any cadmium-rich zinc dust that may be formed in the dephlegmator from entering the cadmium column. Floating metallic dust is removed from 30 time to time through a normally plugged tap hole 27 in the wall of the dephlegmator. A vapor outlet 28 communicates with the top of the dephlegmator.

35 Impure molten zinc metal is introduced into the cadmium column through a pipe 30 communicating with a charging well 31. A continuous stream of molten metal flows into the charging well 31 through an opening 32 in the bottom 40 of a superposed charging well 33. The amount of molten metal flowing through the opening 32 is regulated by adjustment of the position of a cooperating adjustable valve stem 34. An appropriate level of molten metal is continuously 45 maintained in the upper charging well 33. The pipe 30 conveys the molten metal from the charging well 31 into one of the lower trays 20 of the cadmium column.

The bottom of the cadmium column is formed 50 by a tray 35 having a lateral opening communicating with a discharge pipe 36. Molten metal is discharged from the base of the cadmium column through a liquid seal established by a partition wall 37, and is conveyed through the tube 55 36 to the lead-eliminating rectifying column (hereinafter designated lead-column).

The lower portion of the lead column is built 60 within the heating chamber 41 of a furnace structure 40. The heating chamber is provided with burner openings 42 and an outlet 39 for the 65 exhaust heating gases (see Fig. 4). This lower portion of the lead column is built up of trays 44 similar to the trays 14, and the upper portion of the lead column is built up of trays 50 similar to the trays 20. Molten metal is withdrawn from 70 the base of the lead column through a discharge outlet 49. Above the furnace structure 40, the column of trays 50 is surrounded by an appropriate layer of heat insulating material 43.

75 The top of the lead column is connected by an orifice 45 with a zinc oxide combustion chamber 46. The combustion chamber is provided with ports 47 for the entrance of air. The zinc oxide fume produced by combustion of the zinc vapor in the chamber 46 is carried off through a pipe

line 48 to an appropriate zinc oxide collecting device, such for example as a bag house.

Fig. 5 illustrates the connection between the uppermost channeled tray 44 and the lowermost flat-bottomed tray 50. In consequence of the form of these trays, the flat bottom of the lowermost tray 50 approaches very close to the flat portion of the bottom of the uppermost channeled tray 44. Accordingly, the space available for vapor flow between these trays is so constricted as to possibly interfere with the free flow of vapor upwardly through the column. To obviate this difficulty, the opening 51 in the lowermost tray 50 is positioned directly above the opening 52 in the uppermost tray 44. Zinc vapor can thus ascend directly through these two registering openings without passing through the narrow space between the trays. In order to prevent short-circuiting of descending molten metal through these registering openings, the inner edge of the opening 51 of the lowermost tray 50 is provided with an upstanding rib 53 terminating short of each side of the tray, thereby providing openings 54 so positioned that molten metal overflowing the tray is directed into the side channels 55 of the uppermost tray 44 (see Fig. 5). As previously mentioned, a similar arrangement is provided between the corresponding trays in the cadmium column.

In practicing the method of the invention in 30 the apparatus illustrated in the drawing, a continuous stream of molten zinc metal contaminated with lead and cadmium flows through the pipe 30 into one of the trays 20 of the cadmium column. Heat is supplied in controlled amount 35 to the lower portion of the column (by the heating chamber 11) to volatilize the molten metal in amount sufficient to rectify continuously the mixture of zinc and cadmium undergoing the rectification treatment in the column. Metallic vapor 40 ascends the column in intimate contact with the descending molten metal. In consequence of the rectifying action of the column, the ascending vapor becomes progressively enriched in cadmium and the descending (refluxing) molten metal becomes progressively freed of cadmium. A cadmium rich zinc vapor escapes from the top of the column into the dephlegmator 24. All but a cadmium-rich fraction of the vapor entering the dephlegmator is condensed therein and is returned 50 to the rectifying column for the further removal of cadmium therefrom. The cadmium-rich fraction of the vapor uncondensed in the dephlegmator escapes through the pipe 28 to an appropriate recovery device (not shown), such as a canister, condenser, combustion chamber or the like.

Molten zinc metal, purified with respect to cadmium, accumulates in a sump at the base of the cadmium column, and flowing under the curtain wall 37 is delivered by the pipe 36 to the lead 60 column. The wall 37 provides a liquid seal for the discharge of molten metal from the cadmium column into the lead column. This liquid seal is necessary in order to prevent short-circuiting of cadmium-rich vapor into the lead column. If 65 such vapor should enter the lead column, the cadmium therein would accompany and contaminate the purified zinc vapor delivered from the lead column to the zinc oxide combustion chamber.

The pipe 36 delivers molten zinc metal (purified with respect to cadmium) into one of the trays 50 of the lead column in a substantially continuous stream. The lower portion of the lead column is operated in effect as a zinc distilling retort or boiler, being adequately heated for this pur- 75

pose by the hot gases flowing through the heating chamber 41. Metallic vapor ascends the column in intimate contact with descending molten metal. In consequence of the rectifying action of the column, the ascending vapor becomes progressively freed of lead while the descending molten metal becomes progressively enriched in lead. The purified zinc vapor passes from the top of the lead column through the orifice 45 into the combustion chamber 46 where it is oxidized or burned in the presence of air to zinc oxide. The molten metal accumulating at the base of the lead column is high in lead and iron and other impurities with boiling points higher than that of zinc. This impure molten metal is tapped out of the column, either continuously or periodically, through the discharge outlet 49.

While molten metal is discharged from the base of both the cadmium column and the lead column, the lower heated portions of the two columns are operated in different manners. The molten metal discharged from the bottom of the cadmium column consists of zinc contaminated with lead but purified with respect to cadmium. Heat is supplied to the lower portion of the cadmium column in adequate amount to effect continuous rectification of the mixture of zinc and cadmium undergoing treatment in the column. In other words, the base of the cadmium column is not heated with the object of driving off all of the zinc that enters it as vapor. On the other hand, the molten metal delivered at the base of the lead column consists of lead, iron and other impurities with boiling points higher than zinc accompanied by a limited amount of zinc. The purpose in heating the lower portion of the lead column is thus to volatilize as far as practicable all of the zinc that enters it and to deliver the resulting vapor in purified form to the zinc oxide combustion chamber after the vapor has passed through the rectifying column. The lower portion of the lead column is thus operated in effect as a retort or boiler for distilling zinc metal.

While we have hereinbefore specifically described the utilization of the purified zinc vapor in the manufacture of zinc oxide, it is to be understood that the purified zinc vapor may be utilized in any other desired manner, as for example, in the manufacture of zinc dust.

The apparatus illustrated in the drawings as particularly adapted for the practice of the invention may be variously modified in construction and arrangement of operating units without departing from the principles of the invention. In general, the improved apparatus of the invention comprises a cadmium-eliminating rectifying column operatively associated with a lead-eliminating rectifying column so that molten zinc metal purified with respect to cadmium is delivered from the base of the cadmium column to the lead column from which a purified zinc vapor is withdrawn. Various other forms of trans-

verse baffles may be used in place of the trays illustrated in the drawings. When so available the impure zinc contaminated with lead and cadmium may be introduced into the cadmium column in the form of impure vapor rather than impure molten metal. Likewise, cadmium-rich metal may be withdrawn from the dephlegmator at the top of the cadmium column in the form of molten metal instead of vapor.

We claim:

1. The method of producing purified zinc vapor substantially free from cadmium and lead, which comprises introducing molten zinc contaminated with cadmium and lead into a cadmium-eliminating rectifying column, heating said molten zinc within the cadmium-eliminating column by conduction through a wall of the lower portion thereof to vaporize the molten metal at least in part, passing the resulting metal vapor in a substantially undiluted condition in contact with refluxing molten metal within the cadmium-eliminating column, withdrawing cadmium from the top of the cadmium-eliminating column, flowing refluxed molten zinc substantially free of cadmium but contaminated with the lead from the base of the cadmium-eliminating column through a molten metal seal into a lead-eliminating rectifying column, heating the metal within the lead-eliminating column by conduction through a wall of the lower portion thereof to vaporize the zinc in large part, passing the resulting metal vapor in a substantially undiluted condition in contact with refluxing molten zinc within the lead-eliminating column, withdrawing lead from the base of the lead-eliminating column, and withdrawing zinc vapor substantially free from lead and cadmium from the top of the lead-eliminating column.

2. An apparatus for producing zinc vapor substantially free from cadmium and lead, which comprises a cadmium-eliminating rectifying column, means for introducing zinc contaminated with cadmium and lead into the cadmium-eliminating column, a heating chamber adjacent the lower wall portion of the cadmium-eliminating column, means for withdrawing cadmium from the top of the cadmium-eliminating column, a lead-eliminating rectifying column, a conduit connecting the base of the cadmium-eliminating column with the lead-eliminating column, a molten metal seal disposed between the cadmium-eliminating and the lead-eliminating column, a heating chamber adjacent a lower wall portion of the lead-eliminating column, means for withdrawing lead from the base of the lead-eliminating column, and means for withdrawing zinc vapor substantially free from cadmium and lead from the upper end of the lead-eliminating column.

PHILIP MCLEAN GINDER. 60  
WILLIS McGERALD PEIRCE.  
ROBERT KERR WARING.